

Sept. 23, 1952

**W. T. GEYER**

**2,611,693**

## METHOD FOR REFINING MOLTEN METAL

Filed March 31, 1948



Fig. 1.



impurities. INVENTOR.  
Wallace C. Geyer  
BY  
Munn, Fiddy, Blasius & Rich  
Atty's.

## UNITED STATES PATENT OFFICE

2,611,693

## METHOD FOR REFINING MOLTEN METAL

Wallace Thomas Geyer, Mount Rainier, Md.

Application March 31, 1948, Serial No. 18,183

1 Claim. (Cl. 75—58)

1

My invention has for its primary object to provide a method of treating molten pig iron and refining it by first removing the impurities present and subsequently producing from the remaining iron compounds a metallic free iron by the addition of an active element or compound which in turn is removed leaving a free metallic iron capable of being made into suitable alloys, or which can be cast directly into ingots preparatory to rolling, drawing, or forging.

My invention also comprehends the method of operating a suitable apparatus by means of which the foregoing may be accomplished expeditiously in an economical manner in batches received directly from a blast furnace and according to the output desired.

To these and other ends my invention comprises further improvements and advantages as will be further described in the accompanying specification, the novel features thereof being set forth in the appended claim.

In the drawing:

Figure 1 is a side elevation of a retort or crucible shown partly in section illustrating one means by which my invention may be carried out.

Figure 2 is an enlarged vertical section showing the discharge end of the retort.

Similar reference numerals, in the several figures, indicate similar parts.

In carrying out my invention I employ a rotary vessel of heavy construction, such as shown in Fig. 1, comprising an outer circular metallic shell having side walls 10 sloping upwardly and outwardly from a comparatively restricted bottom 11 provided with a controlled recess 12. The inner surface of the side walls and the bottom are protected by a refractory lining 13, the area of the bottom surrounding the opening 12 being dish shaped, or depressed somewhat, as indicated at 14, below the upper or inner end of said opening to form a surrounding shallow well. Extending over the upper end of the vessel is a hood having a depending rim 15 and a conical top 16 from the center of which is an upwardly extending stack 17 containing an exhaust fan 18. At one side of the hood is a charging funnel 19 having a spout 20 discharging close to one side of the vessel.

Extending downwardly from the hood are arms 21 forming a frame work carrying a guide 22 in which is a vertically movable rod 23 which may be raised and lowered by means of a cable 24 trained over a pulley 25 also carried within the hood. The rod carries at its lower end a

2

pointed plug or stopper 26 designed to control the outflow of materials through the opening 12.

I support the retort for high speed rotary movement on a frame work 30, its weight being carried on a bottom ring 31 and an intermediate ring 32 with relation to each of which are corresponding rings 33 and 34 on said frame. The latter each comprise channels in which the rings 31 and 32 are centered in Babbitt bearings whereby not only is the weight of the retort carried on suitable bearings which also serve to prevent its lateral displacement. The upper supporting ring 32 also comprises a laterally projecting horizontal portion which is provided with 15 bevel gear teeth 38 to which power is imparted by a bevel pinion 39 on a shaft 40 driven by a motor 41.

The retort operates as a centrifuge. It is preferably charged while at rest by pouring therein 20 through the funnel 19 a quantity of molten pig iron, received in the state in which it flows from the blast furnace, sufficient to partially fill it to approximately the level indicated by the line A. As the rotary speed of the retort increases the 25 liquid metal moves upwardly along the sloping inner sides of the vessel generating a paraboloid of revolution B. This action, due to the centrifugal power generated in the molten metal, may be derived from Newton's equation.

30

$$F=Ma$$

where

F is the force,

M the mass, and

a the acceleration.

In practice I increase the rotary speed of the vessel until such time as the shape of the inner surface B of the metal at the bottom coincides 40 with the opening of the central orifice 12. Thereafter the speed is maintained constant during the time required for treatment of the batch, or charge, in the manner now to be explained.

It will be realized that this high speed of the 45 retort imparts a force to the molten metal which causes the pure iron particles in the molten mass to move outwardly thus displacing the lighter impurities which may be classified generally as compounds and particularly as those impurities 50 which may remain in pig iron after the slag has been tapped off. These impurities together with occluded gases, I cause to be displaced inwardly to the inner face of the paraboloid. When these impurities arrive at this point they will flow 55 downwardly while the erupting gases thus re-

leased to the air are exhausted upwardly through the stack 17.

The foregoing action may be represented by the following formula in which  $A_n$  represents the normal acceleration of the pure iron particles which exerts a reaction outward force serving to drive the lighter impurities inwardly. Assuming the vessel to be rotating at a constant speed.

$$A_n = \frac{V^2}{r}$$

V the velocity =  $rw$ , the latter character representing the angular velocity created;  $r$  being the radius of the vessel. Wherefore  $A_n = rw^2$ .

Substituting this in the previous formula where  $F = Ma$  the resultant becomes  $F = Mrw^2$  showing that the force applied to the mass introduced into the retort is directly dependent upon the character of such mass, and the distance separate particles thereof are removed from the axis of rotation. Hence, the lighter a particle the less is the resultant force tending to move it outwardly.

When the paraboloid of revolution is created the slag or lighter particles are erupted, or displaced by the heavier pure iron and as they exude become subject to the action of gravity according to the formula:

$$y = \frac{w^2 r^2}{2g}$$

where  $y$  represents the exuded light particles above the vortex;  $w$  the angular velocity;  $r$  the radius of the vessel, and  $g$  the acceleration due to gravity.

The undesired impurities are allowed to escape via the central passage 12 which is opened by elevating the stopper 26.

The second step in carrying out my invention comprises reducing the metallic free iron which I have purified, up to a certain point, as above described by still further removing from it the combined impurities to render it capable of conversion into an alloy. Generally this second step is accomplished by the addition of a more active element or compound to the free iron while the mass is still at the high velocity which maintains its inner surface as a paraboloid.

In carrying out this step of the process I melt a proportional quantity of aluminum and slowly pass it into the funnel 19 the off center spout 20 of which discharges it against the surface B of the molten iron. It will be seen that the aluminum due to its light weight will gravitate slowly along the surface of the molten iron during which time various chemical reactions with the aluminum occur viz.

(a) It, the aluminum, reduces the remaining or ferric oxide oxygen in the mass of iron leaving free iron and  $Al_2O_4$ .

(b) It combines with sulphur converting it into aluminum sulphide.

(c) It combines with the phosphorus forming aluminum phosphide.

(d) Residual gases which are being continued to be expelled from the iron will be absorbed by the molten aluminum.

(e) It combines with the excess carbon creating  $Al_4C_3$ .

(f) After the above reductions have taken place other complex compounds of aluminum and iron will occur and these are likewise removed.

The above chemical reactions are known to produce heat and this is a desirable factor as 75

they tend to maintain, rather than reduce, the temperature of the body of metal undergoing treatment.

When, either empirically, or by observation, it is determined that the reactions have been completed the unwanted expelled compounds are allowed to escape through the bottom exit 12 in the same manner as before described with reference to the slag. Thereafter the stopper 26 is replaced and the vessel is allowed to come to rest.

Since the molten mass has now been freed of substantially all impurities the batch is ready to receive such additional constituents as may be required to convert it into steel of the desired quality, or any desired alloy, following which it may be discharged from the retort and cast into ingots preparatory to forging, rolling or drawing processes.

It will be noted that a particular advantage results from practicing my invention in that since I am able to remove the impurities existing in the pig iron as it is received from the blast furnace to such a substantial extent that at the time when the alloying materials are added it is unnecessary to use any of the counter acting effect substances currently employed in the production of metal alloys.

A still further advantage I am able to obtain results from the fact that the treatment of the molten iron is accomplished without the necessity of maintaining a constant heat under the retort. This is primarily due to the speed with which the impurities are removed and secondarily because of the reaction occurring when the melted aluminum is added which serves to raise the temperature of the mass.

More or less frequently in the treatment of batches of pig iron they will contain a small percentage of other elements or compounds which molecularly are heavier than the iron particles. These are deemed inconsequential for all practical purposes and commercially no attention is paid to them, however, in order to eliminate any possible effect they might have on occasion in the practicing of my invention I provide means in the retort for segregating them. Observing Fig. 2 it will be seen that the inner end of the outlet 12 is elevated slightly above the surrounding bottom of the retort. This arrangement forms a shallow circular depression, or well, in which such heavier substances may be trapped during the rotation of the vessel and as the surface of the well is curved it will be seen that when the batch as a whole is permitted to escape such heavier elements will be held in the retort, from which they may be subsequently removed separately.

I claim:

The method of producing substantially pure iron consisting in centrifuging a mass of molten iron to create an inner paraboloid face thereon, then reducing all compounds of iron in said mass by continuously applying molten aluminum to the upper edge of said paraboloid face allowing said molten aluminum to gravitate slowly along the surface of the revolving mass whereupon said molten aluminum reacts with all compounds of iron in the mass to form the free iron metal, and removing the aluminum compounds from the bottom of the paraboloid face.

WALLACE THOMAS GEYER.

(References on following page)

## REFERENCES CITED

The following references are of record in the file of this patent:

## UNITED STATES PATENTS

| Number    | Name               | Date          |
|-----------|--------------------|---------------|
| 196,204   | Eaton              | Oct. 16, 1877 |
| 399,117   | Adams, Jr., et al. | Mar. 5, 1889  |
| 433,142   | Peck               | July 29, 1890 |
| 811,522   | Seaman             | Jan. 30, 1906 |
| 1,196,829 | Wescott            | Sept. 5, 1916 |

| Number    | Name            | Date          |
|-----------|-----------------|---------------|
| 1,332,585 | White           | Mar. 2, 1920  |
| 1,347,741 | Hadfield        | July 27, 1920 |
| 1,681,191 | Maximoff et al. | Aug. 21, 1928 |
| 2,099,593 | Bender et al.   | Nov. 16, 1937 |
| 2,128,444 | Vroonen         | Aug. 30, 1938 |
| 2,134,905 | Bampfylde       | Nov. 1, 1938  |
| 2,355,362 | Campbell        | Aug. 8, 1944  |
| 2,355,885 | Merle           | Aug. 15, 1944 |
| 2,395,286 | Merle           | Feb. 19, 1946 |
| 2,507,490 | Cohen           | May 16, 1950  |